# EUROPEAN PATENT SPECIFICATION

(11) **EP 0 607 446 B1**
(45) Date of publication and mention of the grant of the patent: **03.02.1999**
(21) Application number: 93910338.8
(22) Date of filing: 13.05.1993
(51) Int. Cl.: C06D 5/00, C06D 5/06, C06B 29/02, C06B 43/00

(54) **GAS GENERATING AGENT FOR AIR BAGS**
GASERZEUGUNGSMITTEL FÜR AIRBAGS
AGENT GENERATEUR DE GAZ POUR SACS GONFLABLES

(30) Priority: 13.07.1992 JP 185251/92; 13.07.1992 JP 185253/92
(43) Date of publication of application: 27.07.1994
(73) Proprietor: NIPPON KOKI CO., LTD., Minato-ku, Tokyo 105 (JP); DAICEL CHEMICAL INDUSTRIES, LTD., Sakai-shi, Osaka 590 (JP); OTSUKA KAGAKU KABUSHIKI KAISHA, Osaka-shi Osaka-fu 540 (JP)
(72) Inventor: YOSHIDA, Tadao, Souka-shi, Saitama 340 (JP)
(74) Representative: Barz, Peter, Dr.
(86) International application number: JP9300634
(87) International publication number: WO9401381

(56) References cited:
- EP-A- 0 482 852
- EP-A- 0 607 450
- DE-A- 2 063 586
- DE-A- 2 351 401
- FR-A- 1 063 438
- JP-A- 2 221 179
- JP-A- 2 221 179
- JP-A- 3 153 593
- JP-A- 4 026 579
- JP-A- 4 265 292
- JP-A-50 083 270
- JP-B-60 028 797
- US-A- 3 214 304
- US-A- 4 358 327
- US-A- 4 386 979
- US-A- 5 125 684

## Description

This invention relates to an air bag gas generating composition.

The so-called air bag system in which a nylon bag stowed in the steering wheel assembly or dashboard of a car is inflated on sensing a car crash occurring at high speed to thereby protect the driver and other passengers against being injured or killed by the impact against the steering wheel or front glass is claiming a phenomenally increasing share of the market reflecting the current rigorous requirements concerning driving safety.

In this air bag system, a gas generating composition is ignited, either electrically or mechanically, in an instant on sensing a car crash to thereby inflate the bag with the gas so generated. The gas generating composition is generally supplied as molded into a pellet or disk form. It is essential that such a gas generating composition insures an appropriate burning velocity. If the burning velocity is too low, the bag cannot be inflated in an instant so that the system fails to achieve its object. The gas generating composition is a powdery composition having the property to get ignited by a shock. Shock ignitability is the sensitivity of a powder to shock ignition and an excessively high shock sensitivity is undesirable from the standpoint of safety because it represents a high risk of explosion in the course of production, e.g. in the mixing stage or in the molding stage. Therefore, shock sensitivity is preferably as low as possible.

It is also necessary that the combustion temperature of the gas generating composition be not too high. This is because, to absorb the shock of a car crash to the driver or passenger and help him to escape, generally the inflated air bag then releases the internal gas to shrink but if the combustion temperature is too high, the released gas is also hot enough to cause the passenger to sustain a burn, perforate the bag to detract from its function, or burn the bag to induce a car fire.

Known air bag gas generating compositions comprise sodium azide as the gas generating base and certain additives such as an oxidizing agent [e.g. metal oxides such as TiO₂, MnO₂, Fe₂O₃, CuO, etc., nitrates such as NaNO₃, KNO₃, Cu(NO₃)₂, etc., perchlorates such as KClO₄, NaClO₄, etc. and chlorates such as KClO₃, NaClO₃, etc.], a reducing metal [Zr, Mg, Al, Ti, etc.], a cooling agent [Na₂CO₃, K₂CO₃, CaCO₃, FeSO₄, etc.], a pH control agent [iron sulfate etc.], a mechanical performance agent [MoS₂, KBr, graphite, etc.] and so on.

Such sodium azide-based gas generating compositions are in common use today partly because the generated gas is nitrogen gas for the most part and partly because they have adequate burning velocities and relatively low combustion temperatures. However, sodium azide has the following disadvantages.
(1) It shows the risk of causing a fire on decomposition or combustion. Thus, since a fire may be induced in the course of production (on mixing with the oxidizing agent, in the final granulation stage, etc.), it requires a rigorous safety control.
(2) It produces Na on decomposition. Since Na reacts with water to generate hydrogen and become ignited to produce a toxic fume, there is considerable difficulty in treatment.
(3) It reacts with the oxidising agent to liberate toxic substances such as Na₂O and its derivatives (such as NaOH), thus calling for careful handling in the course of production.
(4) It is acknowledged that the gas generated on combustion or decomposition of sodium azide is rich in nitrogen and very lean in toxic substances so that there is practically no problem. However, for added safety, a further reduction in the level of toxic substances is desirable.
(5) Crude sodium azide in gas generating compositions is hygroscopic and since the absorption of moisture leads to a decrease in combustibility, there must be an effective provision for the prevention of moisture absorption.
(6) Since it is a toxic and hazardous substance, an additional capital investment is needed for securing safety.

In view of the above disadvantages of sodium aside, the advent has been awaited of an air bag gas generating composition which, compared with the sodium azide-based gas generating composition mentioned above, would have an equivalent or lower shock ignitability, equivalent or higher burning velocity and gas output, and relatively low combustion temperature, and which is lower in the risk of fire and intoxication hazards and lower in costs than the sodium azide-based gas generating composition.

Meanwhile, several attempts have been made to use other nitrogen-containing compounds as the base of a gas generating composition. For example, it has been proposed to subject a reducing metal, such as Zr or Mg, and an oxidizing compound, such as potassium perchlorate or potassium chlorate, to redox reaction to thereby ignite the gas generating base with the resultant heat of reaction. As the gas generating base, smokeless powder, nitrocellulose, azodicarbonamide, aminoguanidine and thiourea have been mentioned (JP-B-9734/74 and 21171/74 and DE-A-2063586). However, the burning velocity that can be obtained by the above method is insufficient for practical application to the air bag. Moreover, since the mixture of reducing metal and oxidizing compound has a very high shock sensitivity, the risk of handling hazards is high. Furthermore, the combustion temperature is also suspected to be too high.

JP-A-118979/75 discloses an air bag gas generating composition comprising a nitrogen-containing compound such as azodicarbonamide, trihydrazinotriazine or the like and an oxidizing agent such as potassium permanganate, manganese dioxide, barium dichromate, barium peroxide or the like. However, the use of potassium permanganate or manganese dioxide as the oxidizing agent does not insure satisfactory shock sensitivity or burning velocity, while the use of barium dichromate or barium peroxide as the oxidizing agent gives rise to toxic substances in the liberated gas.

US-A-5 125 684 discloses a stable extrudable non-azide crash bag propellant composition for generating high quality nitrogen gas and a low temperature process for producing the same from an extrudable mass containing an effective amount of a cellulose-based binder. The disclosed composition contains, as one component, an energetic component selected from nitroguanidine, triaminoguanidine nitrate, ethylene dinitramine, cyclotriethylenetrinitramine, cyclotetramethylenetetranitramine, trinitrotoluene and pentaerythritol tetranitrate.

DE-A-23 51 401 discloses an air bag gas generating composition comprising (i) an alkali or alkaline earth metal azide (e.g. sodium azide), (ii) an alkali metal salt of perchloric acid (or, alternatively, an alkali metal bi-chromate) and (iii) aminotetrazole, hydrated aminotetrazole, azodicarbonamide (ADCA) or azotetrazole. In the disclosed composition, the main component of the gas generating base is a metal azide as the component (i). Moreover, in all examples of said document aminotetrazole is used as component (iii).

US-A-4 386 979 discloses an air bag gas generating composition comprising dicyanodiamide or a similar cyanamide compound and an oxidizer such as an oxo halogen acid salt, a salt of nitric acid or the like. The disclosed gas generating composition involves a high burning temperature in the range of from 1200°C to 1600°C.

It is an object of this invention to provide an air bag gas generating composition having a shock sensitivity either equivalent to or lower than that of the gas generating composition based on sodium azide.

Another object of this invention is to provide an air bag gas generating composition which is either equivalent to or even higher than the sodium azide-based gas generating composition in burning velocity and gas output.

A still further object of this invention is to provide an air bag gas generating composition which is free from the above-mentioned disadvantages (1) through (6) of the azide compound.

It is a further object of this invention to provide an air bag gas generating composition which is low in combustion temperature with a lower risk of fire and intoxication hazards as compared with sodium azide.

The inventor of this invention made an extensive exploration to accomplish the above objects with his attention focused on a nitrogen-containing compound which by itself has very low risks of fire or intoxication hazards due to decomposition or combustion and found that by causing azodicarbonamide to react directly with a defined oxidizing agent, that is a halogen oxo acid salt, taking advantage of the reducing property of the former instead of combusting the nitrogen-containing compound with the heat of a redox reaction, there can be realized not only a shock sensitivity either equivalent to or lower than that of the sodium azide-based gas generating composition but also a burning velocity and a gas output, both of which are either equivalent to or higher than those of said sodium azide-based composition, as well as a practically useful, low combustion temperature.

This invention is, therefore, directed to an air bag gas generating composition consisting of azodicarbonamide and a halogen oxo acid salt in certain relative amounts as given below, as well as certain optional compounds specified hereinbelow.

In accordance with this invention azocarbonamide is used as the gas generation base. There is no limitation on the form or grain size of the azodicarbonamide and a suitable one can be selectively employed.

The oxidizing agent to be used in this invention is a halogen oxo acid salt. As the halogen oxo acid salt, any of the known species can be employed. Preferred are halogenates and perhalogenates and particularly preferred are the corresponding alkali metal salts. The alkali metal halogenates include chlorates and bromates such as potassium chlorate, sodium chlorate, potassium bromate and sodium bromate, among others. The alkali metal perhalogenates include perchlorates and perbromates such as potassium perchlorate, sodium perchlorate, potassium perbromate and sodium perbromate, among others. These halogen oxo acid salts may be used alone or in combination. The amount of the halogen oxo acid salt is generally stoichiometric, that is to say the amount necessary for complete oxidation and combustion of azodicarbonamide based on its oxygen content, but since the burning velocity, combustion temperature and combustion product composition can be freely controlled by varying the ratio of halogen oxo acid salt to azodicarbonamide, its amount can be selected from a relatively broad range, i.e., 20 to 233.3 parts by weight, preferably 20 - 200 parts by weight, more preferably 30 - 200 parts by weight, of the halogen oxo acid salt can be used per 100 parts by weight of azodicarbonamide. The form and grain size of the halogen oxo acid are not particularly critical and can be selected in each case.

The composition of this invention may contain, within the range not affecting its performance characteristics, at least one additive selected from burning control catalysts, antidetonation agents and oxygen donor compounds in addition to said two essential components.

The combustion control catalyst is a catalyst for adjusting the burning velocity, which is one of the basic performance parameters, according to conditions of the intended application, with safety parameters such as low shock ignition and non-detonation properties and other basic performance parameters such as the gas output being fully retained. Such combustion control catalysts include, among others, the oxides, chlorides, carbonates and sulfates of Group IV or Group VI elements of the periodic table of the elements, cellulosic compounds and organic polymers. The oxides, chlorides, carbonates and sulfates of Group IV or VI elements include ZnO, ZnCO₃, MnO₂, FeCl₃, CuO, Pb₃O₄, PbO₂, PbO, Pb₂O₃, S, TiO₂, V₂O₅, CeO₂, Ho₂O₃, CaO₂, Yb₂O₃, Al₂(SO₄)₃, ZnSO₄, MnSO₄, FeSO₄, etc. Among the above cellulosic compounds may be mentioned carboxymethylcellulose and its ether, hydroxymethylcellulose and so on. The organic polymers mentioned above include, among others, soluble starch, polyvinyl alcohol and its partial saponification product, and so on. These combustion control catalysts can be used alone or in combination. The amount of the combustion control catalyst is not critical and can be liberally selected from a broad range. Generally, however, this catalyst is used in a proportion of about 0.1 - 50 parts by weight, preferably about 0.2 - 10 parts by weight, based on 100 parts by weight of azodicarbonamide and said halogen oxo acid salt combined. The grain size of the combustion control catalyst is not critical and can be appropriately selected.

The antidetonation agent is added for preventing the detonation which may occur when the gas generating composition is involved in a fire in the course of production, handling or transportation or subjected to an extraordinary impact. As the addition of such antidetonation agent eliminates the risk of detonation, the safety of the gas-generating composition in various stages of production, handling and transportation can be further enhanced. As the antidetonation agent, a variety of known substances can be utilized. Thus, for example, oxides such as bentonite, alumina, diatomaceous earth, etc. and carbonates and bicarbonates of metals such as Na, K, Ca, Mg, Zn, Cu, Al, etc. can be mentioned. The amount of such antidetonation agent is not critical and can be liberally selected from a broad range. Generally, it can be used in a proportion of about 5 - 30 parts by weight relative to 100 parts by weight of azodicarbonamide and said halogen oxo acid salt combined.

The oxygen donor compound is effective in augmenting the O₂ concentration of the combustion product gas liberated from the composition of this invention. The oxygen donor compound is not critical in kind and a variety of known substances can be employed. For example, CuO₂, K₂O₄, etc. can be mentioned. The amount of the oxygen donor compound is not so critical and can be liberally selected. Generally, however, this donor can be used in a proportion of about 10 - 100 parts by weight based on 100 parts by weight of azodicarbonamide and said halogen oxo acid salt combined.

The composition of this invention may further contain, within the range not affecting its performance characteristics, a combustion temperature control agent and/or a burning velocity control agent. The combustion temperature control agent includes the carbonates and bicarbonates of metals such as Na, K, Ca, Mg, etc., among others. The burning velocity control agent includes the sulfates of Al, Zn, Mn, Fe, etc., among others. The proportion of such combustion temperature control agent and/or burning velocity control agent may generally be about 10 parts by weight, preferably about 5 parts by weight or less, based on 100 parts by weight of azodicarbonamide and said halogen oxo acid salt combined.

The composition of this invention can be manufactured by blending the above-mentioned components. While the resulting mixture as such can be used as the gas generating composition, it may be provided in the form of a molded composition. Such a molded composition can be manufactured by the conventional procedure. For example, the composition of this invention may be mixed with a binder in a suitable ratio and the mixture be molded. The binder may be any binder that is routinely employed. The form of such molded composition is not critical. Thus, it may be a pellet, disk, ball, bar, hollow cylinder, confetti or tetrapod, for instance. It may be solid or porous (e.g. honeycomb-shaped). It is also possible to process each component into a discrete preparation and mix them in use.

The composition of this invention has the following advantages.
(a) The composition of this invention is remarkably low in toxicity and the potential to cause a fire on decomposition or combustion. Therefore, the risk of hazards in handling in the course of production is very low. It can be easily molded, too.
(b) The composition of this invention has a low shock sensitivity which is either equivalent to or lower than that of the sodium azide-based gas generating composition and is, therefore, very safe.
(c) The composition of this invention is equivalent or superior to the sodium azide-based gas generating composition in burning velocity and gas output.
(d) Like the sodium azide-based gas generating composition, the composition of this invention has a relatively low combustion temperature so that it does not have the risk of causing a burn to the passenger or a perforation or burning of the bag. In addition, the level of toxic substances in the product gas is very low.
(e) Since the base nitrogen-containing compound of the composition of this invention (i.e., azodicarbonamide) is not hygroscopic, it is not necessary to provide for the prevention of moisture absorption.
(f) The composition of this invention can be produced at remarkably reduced cost.
(g) Compared with the prior art gas generating compositions, the composition of this invention can be easily disposed of.

### Best Mode of Practicing the Invention

The following examples are intended to describe this invention in further detail. The abbreviation ADCA means azodicarbonamide.

### Example 1

ADCA and halogen oxo acid salt, with or without a combustion control catalyst, were blended according to the formulas shown below in Table 1 to provide compositions (No. 1 - No. 7) of this invention.

Using a hydraulic tablet machine, each of the above compositions of this invention was compressed at 60 kg/cm² to prepare pellets (5 mm in diameter and 5.0 mm high) and each pellet sample was subjected to the 7.5-liter bomb test. The results are shown in Table 2.

### [Bomb (or Vessel) test]

The procedure of the bomb test is now described with reference to Figs. 1 - 3.
1. Weigh out a predetermined amount of the sample (gas generating composition (9), pellets of compositions Nos. 1- 7 of this invention) to place it into a chamber (1).
   The chamber is provided in two sizes. The larger chamber measures 50 mm in inside diameter and is 50 mm high (Fig. 2) and the smaller chamber measures 30 mm in inside diameter and is 50 mm high (Fig. 3).
2. Fit up the chamber with a nozzle having a predetermined diameter (10) and an aluminum rupture plate (11) (0.2 mm thick).
3. Set an ignitor (12) in the reaction chamber. The ignitor comprises a Saran® wrap containing a mixture (2:8) of 0.3 or 1.0 g of boron and KNO₃ and a Ni-Cr wire coil (13) (0.3 mm dia. x 100 mm long) passed through the wrap.
4. Cover the chamber and connect it to a gas trapping bomb (2).
5. Connect ignition leads (4) to electrodes (5) on the bomb cover.
6. Fix the bomb cover (3) on the bomb (2).
7. Connect the measuring circuit wiring.
8. After counting down, energize the ignitor and record the chamber and bomb time-pressure curves and bomb internal temperature.

In Table 2, CPₘₐₓ represents the maximum pressure (kg/cm²) in the reaction chamber, W_{1/2} represents the time (ms) in which the internal pressure of the chamber travels 1/2 of the maximum pressure, BPₘₐₓ represents the maximum pressure (kg/cm²) within the bomb, T₉₀ represents the time (ms) in which the internal pressure of the bomb reaches 90% of the maximum pressure, and BTₘₐₓ represents the maximum temperature (°C) within the bomb. Among these parameters, T₉₀ is a value simulating the inflation time of the air bag. CPₘₐₓ is an index, the values of which indicate that the compositions of this invention retain a satisfactory performance as gas generating compositions. W_{1/2} is a parameter simulating the burning velocity of the gas generating composition within the chamber. BPₘₐₓ is a parameter indicating the gas generating capacity per unit mass of the gas generating composition. BTₘₐₓ is a parameter simulating the temperature of the gas in the fully inflated air bag.

### Example 2

ADCA and halogen oxo acid salt, with or without the combustion control catalyst, were blended according to the formulas (wt. %) shown below in Table 3 to provide compositions of this invention.

Each of the compositions of this invention was subjected to the following shock ignitability (sensitivity) test. As controls, the prior art gas generating compositions (NaN₃-KClO₄-Fe₃O₄ and NaN₃-CuO) were also subjected to the shock ignitiability test.

### [Shock ignitiability test]

This test is designed to measure the degree of readiness of gas generating compositions to be ignited by a shock (shock ignition sensitivity). The experimental procedure is now described with reference to Figs. 4 - 7.
1. [Fig. 4]
   Weigh 5 g of the sample powder (16) into a stainless steel test vessel (15). The vessel (15) is a bottomed cylinder made of stainless steel (SUS 304) and measuring 31 mm in inner diameter, 36 mm in outer diameter, is 2.5 mm thick and 55 mm high.
2. [Fig. 5]
   Place polyethylene cards (17) of required thickness on the sample. The sum of the thicknesses of these polyethylene cards (17) is called the gap length.
3. [Fig. 6]
   Drill a hole, 6.5 mm in diameter, through two 1 mm-thick polyethylene cards (18), set a detonator (19) in the hole and set the assembly in a stainless steel vessel (15). The detonator used was Nippon Kayaku electric detonator No. 0.
4. [Fig. 7]
   For testing any gas generating composition containing a hygroscopic gas generating base (e.g. sodium azide), cover the stainless steel vessel (15) with paraffin (20) for preventing the absorption of moisture.
5. Set this stainless steel vessel securely in a vice in an explosion dome and energize to fire the detonator.
6. Observe whether the sample is ignited or not.
7. If no ignition takes place at the gap length of 1 mm, set 20 g of sample powder (16), insert the detonator D (19) into the sample, place a threaded lid (21) on-the stainless steel vessel (15), and perform the test. By this procedure, even a material with a very low shock sensitivity can be ignited or exploded.

Table 3 shows the ignition limit gap length (ignitable up to that gap length) and the non-ignition limit gap length (not ignitable beyond that gap length).

In this test, a greater critical gap length value represents a higher shock ignition sensitivity. In other words, the greater the critical ignition gap length, the higher is the shock ignition sensitivity and, hence, the risk of hazards.

It is clear from Table 3 that the shock sensitivity of the composition of this invention is equal to or lower than that of the prior art composition, thus being as safe as or safer than the latter.

### Example 3

Azodicarbonamide (abbreviated as ADCA in the following table) and a halogen oxo acid salt, with or without a combustion control catalyst, were blended according to the formulas (wt. %) shown in Table 4 to provide compositions of this invention.

Using a hydraulic tablet machine, each of these compositions was compressed at 60 kg/cm² to prepare pellets (7.6 mm in diameter, 3 mm high) and the pellet sample was subjected to the 7.5-liter bomb test described hereinbefore. The results are shown in Table 4.

As a control, the prior art gas generating composition (NaN₃-CuO) was also subjected to the 7.5-liter bomb test. The results are similarly shown in Table 4.

In this 7.5-liter bomb test, two 0.1 mm - thick aluminum plates were used as the rupture plate to be attached to the chamber cover.

### Example 4

An air bag inflator reactor was loaded with 20 g of pellets (12.3 mm dia. x 3 mm thick) of the composition of this invention comprising 45 parts by weight of azodicarbonamide, 55 parts by weight of sodium chlorate and 2.75 parts by weight of MnO₂ and the loaded inflator was connected to a 28.6-liter tank equipped with a pressure sensor. Using 1 g of B-KNO₃, the pellets were ignited for combustion. The maximum pressure within the tank was 4.3 kgf/cm² gauge and the tank internal pressure rise time associated with combustion of this composition was 50 ms.

As a control, 20 g of pellets (12.3 mm dia. x 3 mm thick) of the gas generating composition suggested by JP-B-21171/74, i.e. a composition comprising 200 parts by weight of azodicarbonamide, 90 parts by weight of sodium chlorate and 10 parts by weight of aluminum, were also subjected to the same tank test. As a result, the rapid combustion of the ignitor alone was observed and the gas generating composition was not as efficiently combusted. Moreover, the maximum ultimate pressure in the tank was as low as 0.3 kgf/cm² gauge.

### Example 5 and 6

Two-hundred (200) parts by weight of azodicarbonamide (abbreviated as ADCA in the following table) was blended with 90 parts by weight of sodium chlorate to provide a composition of this invention.

A control gas generating composition was prepared according to the suggestion made in JP-B 21171/74. Thus, 200 parts by weight of azodicarbonamide was blended with 90 parts by weight of sodium chlorate and 10 parts by weight of Zr powder to provide a control composition.

Each of the above compositions was molded into pellets (5 mm in diameter x 5.0 mm high) in the same manner as Example 1 and the pellet samples were subjected to the following nozzle-pipe combustion test and the shock ignitiability test. The results are shown in Tables 5 and 6.

### [Nozzle-pipe combustion test]

1. Place 5 g of the gas generating composition in a flame-resistant steel vessel (a hollow cylinder measuring 50 mm in inside diameter and being 50 mm high), set a Ni-Cr wire and cover the vessel. The cover is formed with an opening 7 mm in diameter.
2. Apply a voltage of 10 V across the Ni-Cr wire through a Slidac to ignite the gas generating composition.
3. Initially a white smoke emerges from the opening and, then, the composition becomes fired. The flame retention time (combustion time) from the ignition to extinguishment of the flame is visually monitored and, at the same time, recorded with a video camera.

It is apparent from Table 5 that the addition of a reducing metal such as Zr increases the risk potential of a gas generating composition. While the reaction (combustion) of the composition of this invention occurs at low temperature without production of a flame, the Zr-containing control composition is combusted with production of a flame so that the temperature of the product of combustion (gas) is high. It is, therefore, clear that it is not recommendable to add a reducing metal, such as Zr, Al or Mg, to the composition of this invention.

It is clear from Table 6 that the Zr-containing control composition is combusted with production of a flame so that the temperature of the reaction product (gas) is high.

### Example 7

To investigate its combustibility, the composition of this invention was subjected to the strand burner test (cf. "Combustion characteristics of sodium aside gas generating systems", the Proceedings of the 1992 Annual Meeting of the Industrial Explosives Association, Pages 98-99).
1. First, 55 parts by weight of azodicarbonamide was blended with 55 parts by weight of sodium perchlorate and 5 parts by weight of zinc oxide to provide a composition of this invention.
2. This composition was compression-molded into a rectangular piece (8 mm x 5 mm x 50 mm)(pressure: 1.25 t/cm²) and the sides of this piece were coated with a silicone resin to prepare a testpiece with a restriction.
3. The test was performed using a chimney-type strand combustion tester. For measurement, two holes (0.6 mm in diameter) were drilled in the testpiece at a spacing of about 40 mm and after passage of fuses (0.5 mm in diameter), the testpiece was rigidly set in the tester.
4. After the temperature was set to the testing temperature (20°C) in this condition, the testpiece was ignited with a Ni-Cr wire from above for combustion and the burning velocity (mm/sec.) was calculated from the difference between the fusion times of the two fuses and the distance between the holes.
5. The above measurement was carried out under the pressures of 10, 20 and 40 kgf/cm².

The measured burning velocities were 28.3 mm/sec. at 10 kgf/cm², 37.9 mm/s at 20 kgf/cm², and 46.0 mm/s at 40 kgf/cm².

### Example 8

Using the composition of this invention as prepared by blending 30 parts by weight of azodicarbonamide with 70 parts by weight of sodium perchlorate, the burning velocity (mm/sec.) was measured as in Example 8. No ignition occurred at 10 kgf/cm². At 40 kgf/cm², the burning velocity was 48.3 mm/s.

### Example 9

An air bag inflator reactor was loaded with 40 g of pellets (12.3 mm in diameter x 3 mm thick) of the composition of this invention as obtained by blending 45 parts by weight of azodicarbonamide with 55 parts by weight of potassium perchlorate and 10 parts by weight of copper oxide and this inflator was connected to a 28.6-liter tank equipped with a pressure sensor. The pellets were ignited with 1 g of B-KNO₃ for combustion of the composition of this invention. As a result, there was obtained a time-pressure curve similar to that obtained with 80 g of the prior art gas generating composition (NaN₃:KClO₄:Fe₃O₄ = 60:10:30) in a 28.6 liter tank.

### Brief Description of the Drawings

Fig. 1 is a longitudinal section view showing the gas trapping bomb used in the bomb test. Figs. 2 and 3 are diagrammatic illustrations showing the chamber mounted in the gas trapping bomb on exaggerated scale. Figs. 4-7 are diagrammatic representations of the procedure of the shock sensitivity test.
- 1.: Chamber Reactor
- 2.: Gas trapping bomb
- 3.: Bomb cover
- 4.: Leads
- 5.: Electrodes
- 6.: Thermocouple
- 7.: Pressure sensor
- 8.: Gas vent
- 9.: Gas generating composition
- 10.: Nozzle
- 11.: Aluminum rupture plate
- 12.: Ignitor
- 13.: Ni-Cr wire
- 14.: Pressure sensor
- 15.: Stainless steel vessel
- 16.: Sample powder
- 17.: Polyethylene card
- 18.: Polyethylene card
- 19.: Detonator
- 20.: Paraffin
- 21.: Threaded cover

## Claims

1. An air bag gas generating composition consisting of azodicarbonamide, a halogen oxo acid salt and, optionally, at least one member selected from combustion control catalysts, antidetonation agents, oxygen donor compounds, combustion temperature control agents and burning velocity control agents; said halogen oxo acid salt being present in an amount of 20 to 233.3 parts by weight per 100 parts by weight of azodicarbonamide; said composition being free of a reducing metal.

2. The gas generating composition of claim 1 wherein the halogen oxo acid salt is a halogenate and/or a perhalogenate.

3. The gas generating composition of claim 2 wherein the halogenate is an alkali metal halogenate.

4. The gas generating composition of claim 2 wherein the perhalogenate is an alkali metal perhalogenate.

5. The gas generating composition of claim 1 wherein the combustion control catalyst is at least one member selected from the oxides, chlorides and carbonates of Group IV and Group VI elements of the periodic table of the elements.

6. The gas generating composition of claim 1 wherein the combustion control catalyst is at least one member selected from cellulosic compounds and organic polymers.

7. A molded composition consisting of the air bag gas generating composition of any one of claims 1 to 6 and a binder.

8. The molded composition of claim 7 in the form of a pellet, disk, ball, bar, hollow cylinder, confetti or tetrapod.

## Patentansprüche

1. Gaserzeugende Zusammensetzung für Airbags, bestehend aus Azodicarbonamid, einem Halogenoxosäuresalz und gegebenenfalls mindestens einer Substanz ausgewählt aus Verbrennungregelungskatalysatoren, Antidetonationsmitteln, Sauerstoffdonor-Verbindungen, Verbrennungstemperatur-Reguliermifteln und Verbrennungsgeschwindigkeits-Reguliermitteln, wobei das Halogenoxosäuresalz in einer Menge von 20 bis 233.3 Gewichtsteilen pro 100 Gewichtsteile Azodicarbonamid vorliegt und die Zusammensetzung frei von reduzierendem Metall ist.

2. Gaserzeugende Zusammensetzung nach Anspruch 1, worin das Halogenoxosäuresalz ein Halogenat und/oder ein Perhalogenat ist.

3. Gaserzeugende Zusammensetzung nach Anspruch 2, worin das Halogenat ein Alkalimetallhalogenat ist.

4. Gaserzeugende Zusammensetzung nach Anspruch 2, worin das Perhalogenat ein Alkalimetallperhalogenat ist.

5. Gaserzeugende Zusammensetzung nach Anspruch 1, worin der Verbrennungsregelungskatalysator mindestens eine aus den Oxiden, Chloriden und Carbonaten der Elemente der Gruppe IV und der Gruppe VI des Periodensystems der Elemente ausgewählte Substanz ist.

6. Gaserzeugende Zusammensetzung nach Anspruch 1, worin der Verbrennungsregelungskatalysator mindestens eine aus Cellulose-Verbindungen und organischen Polymeren ausgewählte Substanz ist.

7. Geformte Masse, bestehend aus einer gaserzeugenden Zusammensetzung für Airbags nach irgendeinem der Ansprüche 1 bis 6 und einem Bindemittel.

8. Geformte Masse nach Anspruch 7 als Pellet, Scheibe, Kugel, Stab, Hohlzylinder, Dragee oder Tetrapod.

## Revendications

1. Composition générant un gaz pour sacs gonflables comprenant de l'azodicarbonamide, un sel d'halogénooxoacide et éventuellement, au moins un composé choisi parmi des catalyseurs de contrôle de la combustion, des agents anti-détonants, des composés donneurs d'oxygène, des agents pour le contrôle de la température de combustion et des agents pour le contrôle de la vitesse de combustion; ledit sel d'halogéno-oxoacide étant présent en une quantité de 20 à 233,3 parties en poids pour 100 parties en poids d'azodicarbonamide ; ladite composition étant dépourvue d'un métal réducteur.

2. Composition générant un gaz suivant la revendication 1, dans laquelle le sel d'halogéno-oxoacide est un halogénate et/ou un perhalogénate.

3. Composition générant un gaz suivant la revendication 2, dans laquelle l'halogénate est un halogénate de métal alcalin.

4. Composition générant un gaz suivant la revendication 2, dans laquelle le perhalogénate est un perhalogénate de métal alcalin.

5. Composition générant un gaz suivant la revendication 1, dans laquelle le catalyseur de contrôle de la combustion est au moins un composé choisi parmi les oxydes, les chlorures et les carbonates des éléments du Groupe IV et du Groupe VI du tableau périodique des éléments.

6. Composition générant un gaz suivant la revendication 1, dans laquelle le catalyseur de contrôle de la combustion est au moins un composé choisi parmi des composés cellulosiques et des polymères organiques.

7. Composition moulée comprenant la composition générant un gaz pour sacs gonflables suivant l'une quelconque des revendications 1 à 6, et un liant.

8. Composition moulée suivant la revendication 7, sous la forme d'un granulé, d'un disque, d'une bille, d'un barreau, d'un cylindre creux, de confetti ou d'un tétrapode.
